

## UNITED STATES PATENT OFFICE

LINN BRADLEY, OF MONTCLAIR, NEW JERSEY, AND EDWARD P. MCKEEFE, OF PLATTSBURG, NEW YORK, ASSIGNORS TO BRADLEY-MCKEEFE CORPORATION, OF NEW YORK, N. Y., A CORPORATION OF NEW YORK

## PRODUCTION OF WOOD PULP, ETC.

No Drawing.

Application filed September 22, 1925. Serial No. 57,954.

This invention relates to the production of wood pulp from wood and to the treatment of residual liquors from such operations and the production of cooking liquors for use in such operations, etc.

The invention is applicable to a large variety of woods for the production of high grade chemical pulp therefrom for use in the manufacture of papers of various kinds and grades. The invention provides a regenerative process for utilizing the residual liquors for the production of further amounts of cooking liquor. The invention can be carried out in existing mill equipment, such as in the so-called sulphate pulp mills, but without the objectionable odors characteristic of such mills during operation. The invention makes possible the production of high grade pulps possessing good strength and felting properties and with high yields of pulp from various woods, including woods not commonly considered available for the manufacture of high grade chemical pulp.

This application is a continuation in part of our prior applications Serial No. 434,720 filed January 3, 1921, Serial No. 456,187, filed March 28, 1921, Serial No. 481,146, filed June 28, 1921, Serial No. 534,768, filed February 7, 1922, Serial No. 686,137, filed January 14, 1924, Serial No. 704,176, filed April 4, 1924, Serial No. 711,857, filed May 8, 1924, and Serial No. 713,257, filed May 14, 1924.

According to the present invention, the cooking liquor contains caustic soda, sodium sulfite, and sodium sulfid, and the amounts used are such that high grade chemical pulp is produced from the woods treated.

Our investigations indicate that when sodium hydroxide, sodium sulfite and sodium sulfid are utilized together in the cooking liquor the sodium sulfite is less active than when it is used alone or with only small amounts of certain other ingredients; and that it is important for best results to have regulated amounts of the various chemicals present with reference to the wood treated. Our investigations indicate that the activity of sodium sulfite in the presence of sodium sulfid and caustic soda in substantial amounts is only about one quarter the activity of the sodium sulfid

and caustic soda, figured on an equivalent sodium content and we have developed the following hypothetical reaction as possibly indicating the reaction of the sodium sulfite and sodium sulfid when so used:—



The residual liquors from the process contain sodium thiosulfate or other sulfur-containing compounds which readily set free sulphur when treated with acids, and the formation of sodium thiosulfate is theoretically possible in accordance with the above equation. In accordance with this equation it will be noted that half of the sodium enters into combination with organic matter while the other half forms thiosulfate. Assuming that all of the sodium of the sodium sulfid reacts with organic matter, only one quarter of the sodium of the sulfite would so react while the remainder would be present as thiosulfate at the end of the reaction. While we do not desire to limit ourselves by any theoretical explanation of the reactions which take place, nevertheless the above hypothetical reaction seems not an improbable one in the process.

In using the caustic soda, sodium sulfite and sodium sulfid in the cooking liquor, we have used an amount of sodium sulfite in which the sodium content was as much as or more than twice the sodium content of the sodium sulfid; while in other cases we have used cooking liquors in which the sodium present as sulfite was considerably less than the sodium content present as sulfid, e. g., as low as one-half the sodium content present as sulfid.

The sodium hydroxide used in the process can be varied, but is in substantially all cases less than sufficient to satisfactorily pulp the wood if used by itself.

We have found that if the sodium hydroxide, sodium sulfite and sodium sulfid are considered from the standpoint of their sodium content and this content expressed as sodium oxide,  $\text{Na}_2\text{O}$ , the total amount of sodium oxide equivalent of the three ingredients should be such that that of the caustic soda and sodium sulfid, plus one quarter of the sodium

55

60

65

70

75

80

85

90

95

100

oxide equivalent of the sulfite should be in excess of about 12.5%, by weight, of the bone dry weight of the wood treated, e. g., for poplar wood, and in excess of about 15% based on the bone dry weight of the wood for spruce, pines, balsam, etc. Cottonwood appears to require somewhat less than poplar, but nearly all woods require at least as much as poplar, while most of them require somewhat more. An excess of the chemicals can be used, particularly where a quicker cook is desired, and with resinous woods or woods requiring an increased amount of the chemicals. The sodium oxide equivalents figured as above indicated (i. e., the equivalent sodium oxide content of the sodium hydroxide and sodium sulfid plus one-fourth the sodium oxide equivalent of the sodium sulfite) and amounting to 16.5% or more, is sufficient to readily pulp most woods. The amount may be increased e. g. up to 25% or so.

In preparing the cooking liquor we consider that the caustic soda, as above indicated, is all active and in most cases we consider the sodium sulfid as all active, i. e. as entirely available for the chemical reaction of the process, especially when the sodium oxide content of the sodium sulfite present is at least equal to the sodium oxide equivalent of the sodium sulfid present. In calculating the activity of the sodium sulfite, we consider about one-fourth of the sodium oxide content to be active or available in the reaction with the wood substance, so that we take as the total activity one-fourth of the sodium oxide content of the sulfite together with the sodium oxide content of the caustic soda and the sodium oxide equivalent of the sodium sulfid. As an example, for 100 parts of poplar wood by weight (bone-dry basis), and using 12.31 parts of sodium hydroxide, 4 parts of sodium sulfid and 13 parts of sodium sulfite, the activity computed as above is equal to about 14.31% sodium oxide. From this example it is seen that allowance is made for all of the sodium oxide content of the caustic soda and for all of the sodium oxide equivalent of the sodium sulfid and for approximately one-fourth of the sodium oxide content of the sodium sulfite.

When the sodium oxide content of the sodium sulfite is somewhat more than twice the sodium oxide equivalent of the sodium sulfid, the excess sodium sulfite does not appear to be active to any appreciable extent, and allowance is made for only about one quarter of its sodium oxide content, so that this amount of sodium sulfite is equivalent to about one half of the sodium sulfid present. The sodium sulfite is nevertheless important in the process, particularly where there is a relatively high content of sodium sulfid. When sodium thiosulfate is permitted to react with wood it tends to give off elementary sulfur or to form dark colored compounds

unless there is present sufficient sodium sulfite or other sulfur-dissolving compound capable of overcoming this objectionable tendency.

The cooking liquors containing substantial amounts of caustic soda, sodium sulfite and sodium sulfid may advantageously be prepared from the residual liquors of the process, e. g., by concentrating the residual liquors and subjecting them to a calcining or smelting operation with the production of a product from which sodium carbonate and sodium sulfid, with or without sodium sulfite, etc. may be dissolved. The solution containing sodium carbonate and sodium sulfid is advantageously treated with calcium hydroxide or lime and calcium sulfite in admixture with each other and with the amount and proportion of each so chosen as to yield a cooking liquor which will contain the desired amount of caustic soda, sodium sulfite and sodium sulfid. Where the recovered sodium compounds contain a preponderating amount of sodium carbonate and a considerably lesser amount of sodium sulfid, it is easy to prepare such a cooking liquor and to regulate the proportions of the ingredients. By treating part of the solution of the recovered sodium compounds with sulfur dioxide, some of the carbonate may be directly converted into sulfite, and some of the sulfid may be converted into thiosulfate, although by carrying out the sulfiting operating upon the hot liquor the formation of thiosulfate can be minimized. The content of sodium sulfid can to a certain extent be regulated and increased where desired by the addition of sodium sulfate or bisulfate to the residual liquor before the smelting operation. Elementary sulfur may also be dissolved in the causticized solution, or it may be added to the hot solution of sodium carbonate and sodium sulfid before the causticizing and sulfiting treatment; or sulfur may be caused to react with calcium hydroxide and the resulting product utilized for the causticizing treatment. Sodium sulfite can be produced directly from sodium carbonate and sulfur dioxide and added to the cooking liquor. Where sulfur is added to a caustic soda solution it is desirable in some cases to add it to caustic soda which does not contain sodium sulfite and to add the resulting solution to the sodium sulfite containing liquor so as to reduce the tendency of sodium sulfite to react with sulfur to form thiosulfate. Sodium thiosulfate may, however, be present in the cooking liquor, particularly where the amount of sodium sulfite is sufficiently high. The invention will be further illustrated by the following specific examples, carried out with various woods, both deciduous and coniferous, and with cooking liquors of varying composition and activity, but all containing caustic soda, sodium sulfite and so-

dium sulfid in substantial amounts. These cooking liquors have been used in cooking the woods indicated, using a sufficient amount of liquor to submerge the chips and carrying out the cooking operations at a temperature corresponding to a saturated steam pressure of 110 to 120 pounds gauge. The period of heating to bring the charge up to pressure was about two hours and the cook was continued for about three and one-half to five and one-half hours, or until the cooking operation had been completed and the fibres became readily separable.

The cooking liquors are given in the following examples in tabulated form, showing the actual parts by weight of caustic soda, sodium sulfid and sodium sulfite used, together with the parts by weight of wood (figured on bone-dry basis) and the particular wood or mixture of woods treated. At the top of each series of three examples the activity of the cooking liquor is indicated in percentage of sodium oxide and sodium sulfid equivalent based on the bone dry weight of the wood. The sodium oxide and sodium sulfid equivalents are calculated as hereinbefore described. That is, in calculating the sodium oxide equivalent, the sodium oxide content of the caustic soda is taken, together with the sodium oxide equivalent of the sodium sulfid, and one quarter of the sodium oxide content of the sodium sulfite. The sodium sulfid equivalent corresponds molecularly to the sodium oxide equivalent. These equivalents are used as a convenient means of expressing the activity of the cooking liquor with reference to the bone dry weight of the wood.

| Computed activity       |                                 |                        |                          |                        |                       |
|-------------------------|---------------------------------|------------------------|--------------------------|------------------------|-----------------------|
| Na <sub>2</sub> O<12.72 |                                 | Na <sub>2</sub> O<14.0 |                          | Na <sub>2</sub> O<15.3 |                       |
|                         | Na <sub>2</sub> S<16.           | Na <sub>2</sub> S<17.6 | Na <sub>2</sub> S<19.2   | Na <sub>2</sub> O<14.0 | Na <sub>2</sub> S<16. |
| 40                      |                                 |                        |                          |                        |                       |
|                         | NaOH                            | Ex. 1                  | Ex. 4                    | Ex. 7                  |                       |
|                         | 4.313                           | 4.750                  | 5.003                    | 5.756                  |                       |
|                         | Na <sub>2</sub> S               | 8.429                  | 9.264                    | 9.756                  |                       |
|                         | Na <sub>2</sub> SO <sub>3</sub> | 6.797                  | 7.483                    | 7.889                  |                       |
|                         | B. D. wood                      | 85.0 poplar            | 85.5 poplar              | 82.5 poplar            |                       |
|                         |                                 | Ex. 2                  | Ex. 5                    | Ex. 8                  |                       |
|                         | NaOH                            | 4.014                  | 4.416                    | 4.646                  |                       |
|                         | Na <sub>2</sub> S               | 7.814                  | 8.593                    | 9.055                  |                       |
|                         | Na <sub>2</sub> SO <sub>3</sub> | 12.634                 | 13.880                   | 14.614                 |                       |
| 45                      | B. D. wood                      | 85.0 poplar            | 85.5 poplar              | 82.5 poplar            |                       |
|                         |                                 | Ex. 3                  | Ex. 6                    | Ex. 9                  |                       |
|                         | NaOH                            | 3.508                  | 3.853                    | 4.060                  |                       |
|                         | Na <sub>2</sub> S               | 6.847                  | 7.519                    | 7.921                  |                       |
|                         | Na <sub>2</sub> SO <sub>3</sub> | 22.115                 | 24.319                   | 25.589                 |                       |
|                         | B. D. wood                      | 85.0 poplar            | 85.5 poplar              | 82.5 poplar            |                       |
|                         |                                 | Ex. 10                 | Ex. 13                   | Ex. 16                 |                       |
|                         | NaOH                            | 6.785                  | 6.278                    | 7.057                  |                       |
|                         | Na <sub>2</sub> S               | 13.232                 | 6.107                    | 6.865                  |                       |
|                         | Na <sub>2</sub> SO <sub>3</sub> | 10.666                 | 4.939                    | 5.541                  |                       |
| 50                      | B. D. wood                      | 89.5 pine              | 81.2 poplar<br>and birch | 83.0 poplar            |                       |
|                         |                                 | Ex. 11                 | Ex. 14                   | Ex. 17                 |                       |
|                         | NaOH                            | 6.302                  | 5.915                    | 6.655                  |                       |
|                         | Na <sub>2</sub> S               | 12.278                 | 5.777                    | 6.494                  |                       |
|                         | Na <sub>2</sub> SO <sub>3</sub> | 19.842                 | 9.326                    | 10.494                 |                       |
|                         | B. D. wood                      | 89.5 pine              | 81.2 poplar<br>and birch | 83.0 poplar            |                       |
| 55                      |                                 |                        |                          |                        |                       |
|                         | Ex. 12                          | Ex. 15                 | Ex. 18                   | Ex. 17                 |                       |
|                         | NaOH                            | 5.509                  | 4.904                    | 5.903                  |                       |
|                         | Na <sub>2</sub> S               | 10.741                 | 4.867                    | 5.846                  |                       |
|                         | Na <sub>2</sub> SO <sub>3</sub> | 34.717                 | 15.714                   | 18.874                 |                       |
| 60                      | B. D. wood                      | 89.5 pine              | 76.0 poplar<br>and birch | 83.0 poplar            |                       |
|                         |                                 | Ex. 19                 | Ex. 22                   | Ex. 25                 |                       |
|                         | Na <sub>2</sub> O<15.3          | Na <sub>2</sub> O<19.1 | Na <sub>2</sub> O<19.1   | Na <sub>2</sub> O<19.1 |                       |
|                         | Na <sub>2</sub> S<19.2          | Na <sub>2</sub> S<24.  | Na <sub>2</sub> S<24.    | Na <sub>2</sub> S<24.  |                       |
|                         | NaOH                            | 8.12                   | 10.144                   | 10.144                 |                       |
|                         | Na <sub>2</sub> S               | 7.914                  | 9.858                    | 9.856                  |                       |
|                         | Na <sub>2</sub> SO <sub>3</sub> | 6.384                  | 7.978                    | 7.989                  |                       |
| 65                      | CB. D. wood                     | 87.5 poplar            | 87.5 poplar              | 87.5 spruce            |                       |

## Computed activity—Continued

|  |                                 |                          |                        |                        |
|--|---------------------------------|--------------------------|------------------------|------------------------|
|  | Ex. 20                          | Ex. 23                   | Ex. 26                 |                        |
|  | NaOH                            | 7.653                    | 9.573                  | 9.573                  |
|  | Na <sub>2</sub> S               | 7.459                    | 9.334                  | 9.339                  |
|  | Na <sub>2</sub> SO <sub>3</sub> | 12.062                   | 15.083                 | 15.078                 |
|  | B. D. wood                      | 87.5 poplar              | 87.5 poplar            | 87.5 spruce            |
|  |                                 | Ex. 21                   | Ex. 24                 | 70                     |
|  | NaOH                            | 6.901                    | 7.485                  | 8.613                  |
|  | Na <sub>2</sub> S               | 6.714                    | 7.307                  | 8.399                  |
|  | Na <sub>2</sub> SO <sub>3</sub> | 21.719                   | 23.587                 | 27.146                 |
|  | B. D. wood                      | 87.5 poplar              | 76.0 poplar            | 87.5 spruce            |
|  |                                 | Na <sub>2</sub> O<12.9   | Na <sub>2</sub> O<14.0 | Na <sub>2</sub> O<15.3 |
|  | Na <sub>2</sub> S<16.18         | Na <sub>2</sub> S<17.6   | Na <sub>2</sub> S<17.6 | Na <sub>2</sub> S<19.2 |
|  |                                 | Ex. 28                   | Ex. 31                 | 75                     |
|  | NaOH                            | 8.03                     | 9.143                  | 9.982                  |
|  | Na <sub>2</sub> S               | 4.701                    | 5.356                  | 5.848                  |
|  | Na <sub>2</sub> SO <sub>3</sub> | 3.803                    | 4.327                  | 4.733                  |
|  | B. D. wood                      | 81.2 poplar<br>and birch | 85.0 poplar            | 85.0 poplar            |
|  |                                 | Ex. 29                   | Ex. 32                 | 80                     |
|  | NaOH                            | 7.705                    | 8.775                  | 9.568                  |
|  | Na <sub>2</sub> S               | 4.508                    | 5.132                  | 5.609                  |
|  | Na <sub>2</sub> SO <sub>3</sub> | 7.275                    | 8.308                  | 9.042                  |
|  | B. D. wood                      | 81.2 poplar<br>and birch | 85.0 poplar            | 85.0 poplar            |
|  |                                 | Ex. 30                   | Ex. 33                 | 85                     |
|  | NaOH                            | 7.096                    | 8.073                  | 8.809                  |
|  | Na <sub>2</sub> S               | 4.150                    | 4.729                  | 5.147                  |
|  | Na <sub>2</sub> SO <sub>3</sub> | 13.399                   | 15.263                 | 16.652                 |
|  | B. D. wood                      | 81.2 poplar<br>and birch | 85.0 poplar            | 85.0 poplar            |

Cooking liquor No. 1 contains about the minimum activity, computed as hereinbefore described. That is, all of the Na<sub>2</sub>O of the NaOH and the Na<sub>2</sub>S (on a Na<sub>2</sub>O equivalent basis) and one fourth of the Na<sub>2</sub>O content of the Na<sub>2</sub>SO<sub>3</sub>, when added together equal about 16% Na<sub>2</sub>S equivalent, or about 12.72% Na<sub>2</sub>O, based on the bone dry weight of the wood treated. When the amount of Na<sub>2</sub>S is so high and the NaOH and the Na<sub>2</sub>SO<sub>3</sub> are in the proportion given in this example, this wood is fairly well cooked. This same liquor upon cottonwood operates a little better than it does on poplar. There is not quite enough Na<sub>2</sub>SO<sub>3</sub> to yield a light colored pulp. For cooking resinous woods, the chemicals may be used in the same ratio but are advantageously increased in amount so that the activity as computed above is at least 19.2% Na<sub>2</sub>S equivalent, or 15.26% Na<sub>2</sub>O, on the B. D. wood weight.

Cooking liquor No. 2 contains NaOH and Na<sub>2</sub>S in the same ratio as No. 1, but differs therefrom in having an equal amount of Na<sub>2</sub>O equivalent in the sulfite as there is in the sulfid instead of one-half as much as shown in Example No. 1, and the amount of NaOH and of Na<sub>2</sub>S has been slightly reduced so that the activity as computed herein remains substantially the same as in No. 1. This cooking liquor works somewhat better than the cooking liquor No. 1. For coniferous woods it is advantageous to increase the amount of chemicals so that the activity is at least equal to 19.2% Na<sub>2</sub>S equivalent, or 15.26% Na<sub>2</sub>O, on the B. D. weight of the wood (calculated as above).

Cooking liquor No. 3 has the same NaOH—Na<sub>2</sub>S ratios as No. 1 and No. 2 and the amount of chemicals is such that the computed activity is about the same, while the Na<sub>2</sub>SO<sub>3</sub> content is so increased that it contains twice as much Na<sub>2</sub>O equivalent as the Na<sub>2</sub>S. This cooking liquor works better than No. 1 and

No. 2. Where the  $\text{Na}_2\text{S}$  content is relatively high in comparison with the  $\text{NaOH}$ , it is desirable to have a relatively high content of  $\text{Na}_2\text{SO}_3$  so as to lessen the odors developed during cooking, to obtain lighter colored pulp and to furnish a higher content of  $\text{Na}_2\text{S}$  in the recovered soda than would be obtained if the  $\text{Na}_2\text{SO}_3$  content were kept low. An even greater amount of  $\text{Na}_2\text{SO}_3$  can be used than in cooking liquors like No. 3. Cooking liquor having such ratios as in Example No. 3 are very suitable for producing high quality stock provided the activity as computed is kept sufficiently high. By keeping the ratio of  $\text{NaOH}$ — $\text{Na}_2\text{S}$ — $\text{Na}_2\text{SO}_3$  about constant, but increasing the amounts of each in proportion so that the computed activity is at least 18%  $\text{Na}_2\text{S}$  equivalent, or 14.31%  $\text{Na}_2\text{O}$ , for deciduous woods, and at least equal to 19.2%  $\text{Na}_2\text{S}$  equivalent, or 15.26%  $\text{Na}_2\text{O}$  for coniferous woods, excellent pulps, possessing splendid strength and of good color may be readily obtained.

It will be noted that in the cooking liquors of Examples No. 1, No. 2 and No. 3, the  $\text{Na}_2\text{O}$  content of the  $\text{NaOH}$  is substantially one half the  $\text{Na}_2\text{O}$  content (equivalent) of the  $\text{Na}_2\text{S}$ , and that the amount of  $\text{Na}_2\text{SO}_3$  compared with the  $\text{Na}_2\text{S}$  is changed so that it varies from one half as much  $\text{Na}_2\text{O}$  content up to twice as much  $\text{Na}_2\text{O}$  content. It may also be pointed out that with such high  $\text{Na}_2\text{S}$  content it is advantageous to use a relatively high content of  $\text{Na}_2\text{SO}_3$ , and, in fact, even an excess over the equation referred to previously; and that an activity of at least 18%  $\text{Na}_2\text{S}$  equivalent for deciduous woods is desirable in most instances, and an activity of at least 19.2%  $\text{Na}_2\text{S}$  equivalent is desirable for coniferous woods.

In cooking liquors No. 4, No. 5, and No. 6, the ratio of  $\text{NaOH}$  to  $\text{Na}_2\text{S}$  is the same as in those numbered 1, 2 and 3, and the  $\text{Na}_2\text{SO}_3$  varies in amount, e. g. in No. 4 having one half as much  $\text{Na}_2\text{O}$  as there is in the  $\text{Na}_2\text{S}$ , in No. 5 having an equal amount and No. 6 having twice as much  $\text{Na}_2\text{O}$  as the  $\text{Na}_2\text{S}$ . These three cooking liquors differ from the first three in having a higher computed activity, this being equivalent to about 17.6%  $\text{Na}_2\text{S}$ , or 14.00%  $\text{Na}_2\text{O}$ . That of No. 4 has less total sodium than either No. 5 or No. 6, for the same computed activity. No. 6 has a higher content of  $\text{Na}_2\text{SO}_3$  and has been found to yield pulps of somewhat lighter color than No. 4 and even than No. 5.

Cooking liquors Nos. 7, 8 and 9 have the same ratio of  $\text{NaOH}$  to  $\text{Na}_2\text{S}$  as in cooking liquors Nos. 1 to 6, i. e. one half as much  $\text{Na}_2\text{O}$  in the form of  $\text{NaOH}$  as there is in the form of  $\text{Na}_2\text{S}$ , with the  $\text{Na}_2\text{O}$  in the  $\text{Na}_2\text{SO}_3$  ranging from one half the  $\text{Na}_2\text{O}$  of the  $\text{Na}_2\text{S}$ , through an equal amount up to twice as much  $\text{Na}_2\text{O}$  in the  $\text{Na}_2\text{SO}_3$  as there is in the  $\text{Na}_2\text{S}$ . The computed activity in 7, 8 and 9 is sub-

stantially equivalent to 19.2%  $\text{Na}_2\text{S}$ , or to 15.26%  $\text{Na}_2\text{O}$ . An excess of  $\text{Na}_2\text{SO}_3$  over that in No. 9 may be used. A high  $\text{Na}_2\text{SO}_3$  content of the cooking liquor tends to yield a recovered soda product from the furnaces which contains a fairly high percentage of  $\text{Na}_2\text{S}$  which may be retained in the regenerated cooking liquor. This feature is of particular importance where the soda losses are rather high and either  $\text{Na}_2\text{SO}_3$  or  $\text{NaOH}$  or both are used for making up the losses of soda instead of sodium sulfate or nitre cake additions to the cycle.

In cooking liquors Nos. 10, 11 and 12 the ratios of  $\text{NaOH}$  to  $\text{Na}_2\text{S}$  and to  $\text{Na}_2\text{SO}_3$  are seen to be similar to those in 1, 2, 3, in 4, 5, 6, and in 7, 8 and 9, respectively, but the amounts of each reagent have been increased so that the computed activity is up to an equivalent of 25%  $\text{Na}_2\text{S}$ , or 19.08%  $\text{Na}_2\text{O}$ , calculated as above. This strength of cooking liquor, i. e. an equivalent of 24%  $\text{Na}_2\text{S}$  or 19.08%  $\text{Na}_2\text{O}$  on the weight of the bone dry wood makes a very effective cooking liquor for resinous woods and other woods which require a relatively high activity as compared with poplar, cottonwood, birch, maple, beech, etc. Very highly resinous or "fatty" pines have been successfully reduced by each of these cooking liquors (Nos. 10, 11 and 12) and produced a strong and relatively light colored pulp.

In cooking liquors Nos. 13, 14, 15, 16, 17, 18, 19, 20, 21, 22, 23, 24, 25, 26 and 27, the  $\text{NaOH}$  is substantially equivalent to the  $\text{Na}_2\text{S}$ , while the activity in the first three, calculated as above, is equivalent to about 16%  $\text{Na}_2\text{S}$ , the activity in the second three, (16, 17 and 18) is equivalent to about 17.6%  $\text{Na}_2\text{S}$ , in the third group (19, 20 and 21) the activity is equivalent to about 19.2%  $\text{Na}_2\text{S}$ , and in the two latter groups (22 to 27) the activity, as computed herein, is equivalent to about 24%  $\text{Na}_2\text{S}$  on the bone dry weight of the wood. The amount of  $\text{Na}_2\text{O}$  in the  $\text{Na}_2\text{SO}_3$  in each group of three cooking liquors ranges from one half as much  $\text{Na}_2\text{O}$  as is in the  $\text{Na}_2\text{S}$ , through an equal amount up to twice as much  $\text{Na}_2\text{O}$  in the  $\text{Na}_2\text{SO}_3$  as there is in the  $\text{Na}_2\text{S}$ . An even greater amount of  $\text{Na}_2\text{SO}_3$  may be used.

These activities, expressed as above, range from about the lowest point which will satisfactorily cook wood in a single stage operation up to and including sufficient activity for cooking practically all woods which will be used in chemical pulp mills. The  $\text{NaOH}$  content of the liquor is equivalent to the  $\text{Na}_2\text{S}$  content in each example, while the  $\text{Na}_2\text{SO}_3$  is varied in proportion. The higher activities are the ones which will generally be used for resinous woods and other woods which require a high activity to satisfactorily pulp them. When the lower activities are used, we have found that the ones which have the higher amounts of  $\text{Na}_2\text{SO}_3$  give some-

what lighter colored pulps than do those in which the  $\text{Na}_2\text{O}$  content present as  $\text{Na}_2\text{SO}_3$  is less than equal to the  $\text{Na}_2\text{O}$  content present as  $\text{Na}_2\text{S}$ , as the higher  $\text{Na}_2\text{SO}_3$  content generally produces a lighter colored and better stock. These liquors are somewhat milder than those which contain higher percentages of  $\text{NaOH}$  and of  $\text{Na}_2\text{S}$  and less amounts of  $\text{Na}_2\text{SO}_3$ .

- 10 Cooking liquors Nos. 28, 29, 30, 31, 32, 33, 34, 35 and 36 are liquors in which the amount of  $\text{Na}_2\text{O}$  present as  $\text{NaOH}$  is materially greater than the  $\text{Na}_2\text{O}$  equivalent of the  $\text{Na}_2\text{S}$ , and the activity as computed herein 15 ranges from 16.18%  $\text{Na}_2\text{S}$  equivalent through 17.6%  $\text{Na}_2\text{S}$  equivalent and includes three examples in which the activity is 19.2%  $\text{Na}_2\text{S}$  equivalent. The  $\text{Na}_2\text{SO}_3$  ranges from an  $\text{Na}_2\text{O}$  content of one half that of the  $\text{Na}_2\text{S}$  20 through an equal amount up to and including an amount which is twice the  $\text{Na}_2\text{O}$  content of the  $\text{Na}_2\text{S}$ . An even greater amount of  $\text{Na}_2\text{SO}_3$  may be used and this is advantageous especially when the lower activities are 25 employed and it is desired to obtain pulp of lighter color.

In the last nine examples it will be noted that less  $\text{Na}_2\text{S}$  is used and also less  $\text{Na}_2\text{SO}_3$  than the previous examples since more cooking 30 is due to the  $\text{NaOH}$  content. In cases where the  $\text{NaOH}$  predominates over both the  $\text{Na}_2\text{S}$  and  $\text{Na}_2\text{SO}_3$  the amount of chemicals in the digester charge is generally less than is charged when a lower percentage of 35  $\text{NaOH}$  is used. Care should be taken, however, to keep the actual  $\text{NaOH}$  down below the point where the fibres are readily destroyed or objectionably injured.

The process of the present invention is advantageously carried out as a regenerative process by treating the residual liquors of the process for the production of further amounts of cooking liquors therefrom. The residual liquors can be treated according to 40 methods described in our prior applications hereinbefore referred to, e. g., by concentrating the residual liquor, subjecting it to a calcining or smelting operation with resulting production of a product containing 45 sodium sulfid and sodium carbonate, either with or without sodium sulfite etc., and this product can be dissolved or extracted to form a solution which can be treated to produce the cooking liquor. The solution can be treated, e. g., with calcium sulfite, to convert 50 sodium carbonate into sodium sulfite, or with a mixture of calcium sulfite and calcium hydroxide to produce both sodium sulfite and 55 caustic soda in regulated amounts. The solution can also be treated by various other procedures described in our said prior applications for the production of cooking liquors 60 containing sodium sulfide, sodium sulfite, and 65 caustic soda, in regulated amounts, either

with or without the production of sodium thiosulfate, etc.

We claim:

1. The method of producing wood pulp from wood which comprises cooking the wood 70 in a cooking liquor comprising substantial amounts of sodium hydroxide, sodium sulfid and sodium sulfite, the sodium oxide content of the sulfite being greater in amount than the sodium oxide equivalent of the hydroxide. 75

2. The method of producing wood pulp from wood which comprises cooking wood in a cooking liquor comprising substantial amounts of sodium hydroxide sodium sulfid 80 and sodium sulfite, the sodium oxide content of the sulfite being greater than the sodium oxide equivalent of both the sulfid and the hydroxide.

3. The method of producing wood pulp 85 from wood which comprises cooking the wood in a cooking liquor comprising sodium hydroxide, sodium sulfid and sodium sulfite each of which constitutes a principal digesting reagent, the sodium oxide content of the sulfite being more than one-half and less than twice that of the sulfide, the activity, calculated as herein described, being at least 12.5%  $\text{Na}_2\text{O}$ , but less than 14%  $\text{Na}_2\text{O}$ , substantially as described. 90

4. The method of producing wood pulp from wood which comprises cooking the wood in a cooking liquor comprising sodium hydroxide, sodium sulfid and sodium sulfite 100 each of which constitutes a principal digesting reagent, the sodium oxide content of the sulfite being more than one-half and less than twice that of the sulfide, the activity, calculated as herein described, being at least 12.5%  $\text{Na}_2\text{O}$ , but less than 15.26%  $\text{Na}_2\text{O}$ , substantially as described. 105

5. The method of producing wood pulp from wood which comprises cooking the wood in a cooking liquor comprising sodium hydroxide, sodium sulfid and sodium sulfite 110 each of which constitutes a principal digesting reagent, the sodium oxide content of the sulfite being more than one-half and less than twice that of the sulfide, the activity, calculated as herein described, being at least 12.5%  $\text{Na}_2\text{O}$ , but less than 16.53%  $\text{Na}_2\text{O}$ , substantially as described. 115

6. The method of producing wood pulp from wood which comprises cooking the wood in a cooking liquor comprising sodium hydroxide, sodium sulfid and sodium sulfite 120 each of which constitutes a principal digesting reagent, the sodium oxide content of the sulfite being more than one-half and less than twice that of the sulfide, the activity, calculated as herein described, being at least 12.5%  $\text{Na}_2\text{O}$ , but less than 25%  $\text{Na}_2\text{O}$ , substantially as described. 125

7. The method of producing pulp from wood which comprises digesting wood by 130

means of a liquor containing substantial amounts of caustic soda, sodium sulfite and sodium sulfid, the activity of which shall be not less than 12½% as defined above, and said liquor shall include not less than two molecules of sodium sulfite ( $Na_2SO_3$ ) for each molecule of sodium hydroxide ( $NaOH$ ).

8. Method of producing wood pulp from wood, which comprises cooking the wood in 10 a cooking liquor comprising substantial amounts of sodium hydroxide, sodium sulfide and sodium sulfite, the sodium oxide content of the sulfite being greater in amount than the sodium oxide equivalent of either 15 the hydroxide or the sulfide and the sulfide being not less in amount than the hydroxide.

9. The method of producing pulp from wood which comprises digesting wood by means of a liquor containing substantial 20 amounts of sodium sulfite, sodium sulfide, and sodium hydroxide, the sodium oxide equivalent of neither the sulfide nor the hydroxide being less than one-half nor more than equal to the sodium oxide equivalent 25 of the sulfite, and the activity calculated as herein described in excess of about 12.50%.

In testimony whereof we affix our signatures.

LINN BRADLEY.

EDWARD P. MCKEEFE.